

Aug. 19, 1941.

E. J. HALL

2,252,714

PROCESS AND APPARATUS FOR MAKING METAL POWDER

Filed June 29, 1937

2 Sheets-Sheet 1



Aug. 19, 1941.

**E. J. HALL**

2,252,714

# PROCESS AND APPARATUS FOR MAKING METAL POWDER

Filed June 29, 1937

2 Sheets-Sheet 2



INVENTOR  
EVERETT J. HALL, DECEASED  
PER HARRIET L. HALL, EX'TRIX.  
BY Ramsey, Kent, Chisholm & Ledyard  
ATTORNEYS

Patented Aug. 19, 1941

2,252,714

# UNITED STATES PATENT OFFICE

2,252,714

## PROCESS AND APPARATUS FOR MAKING METAL POWDER

Everett J. Hall, deceased, late of Elizabeth, N. J.,  
by Harriet L. Hall, executrix, Elizabeth, N. J.,  
assignor to Metals Disintegrating Company,  
Inc., Union Township, Union County, N. J., a  
corporation of New Jersey

Application June 29, 1937, Serial No. 150,934

16 Claims.

(Cl. 75—72)

This invention relates to the production of copper powder by reducing oxides of copper and then breaking up the resultant friable mass of metallic copper. While not restricted thereto, the invention is particularly adapted to the production of copper powder for bronze bearings and other molded objects.

In manufacturing bearings from copper powder, other materials (e. g. tin and/or graphite) are often mixed with the copper. Large producers of bearings use automatic pressing machinery equipped with automatic filling devices. To insure uniform bearings and continuous performance of the pressing machinery, the bearing material must have requisite flowability. Additionally, the compressibility of the material under the molding pressure must be uniform. After the bearing has been molded, it is sintered or heat treated; and the size of the bearing is changed by this manufacturing step. If the heat treated bearing is too short it must be scrapped; if it is too long, it must be ground down, as the bearing material does not machine satisfactorily. Thus, the bearing material must be such that a uniform and predetermined change of size will take place when the bearing is sintered. Furthermore, the finished bearing must have sufficient strength; and the bearing material must be such as will give the strength.

From the foregoing it will be seen that the bearing manufacturer requires a copper powder which is exceedingly uniform as to the various physical characteristics that affect the manufacture of the bearing. And these physical characteristics must be correlated with the pressing dies, filling machinery, other ingredients added by the bearing manufacturer, size and type of bearing to be made, etc. The result is that the manufacturer of the copper powder is called upon to meet a wide range of powder specifications submitted by bearing manufacturers; and as to each specification a uniform powder must be supplied.

Heretofore copper powder has been made in batches. Trays containing thin layers of oxides of copper were placed in a chamber or furnace which was then closed and reducing gas passed therethrough. After the reduction had been effected the resultant copper powder (and the batch chamber) had to be cooled sufficiently to prevent the powder from being oxidized by contact of the air.

This prior art batch procedure is inefficient and wasteful because (a) to get the desired degree of completeness of reduction of the oxides, the reducing gas must be discharged before its reducing constituents are substantially oxidized, (b) the batch reducing furnace cannot be recharged immediately, but must be first cooled, and (c) there is a large net heat loss due to the

cooling of the batch furnace necessary to reduce the temperature of the newly formed copper powder below the oxidation point. Furthermore, the batch procedure is limited as to the control of the reduction obtainable to produce powder to meet different specifications, and to produce a powder which uniformly meets a given specification.

Among the general objects of the present invention are to provide a more efficient and economical process for reducing copper oxides to form copper powder, to provide a process which can be adequately varied to produce powder to meet different specifications, to provide a process which can be adequately controlled to produce copper powder having uniform predetermined characteristics, and to provide apparatus suitable for such improved processes.

Various specific and detailed objects of the invention will be apparent to those skilled in the art from the disclosure herein of the preferred form of the invention.

In its preferred form the invention comprises a process of continuously reducing oxides in a muffle furnace, but the improvement is not merely that ordinarily obtained by changing from batch procedure to continuous procedure. In various other manufacturing lines batch processes have been quickly replaced by continuous processes, but that has not been the case with the manufacture of copper powder by the reduction of copper oxides. The reduction of copper oxide requires treatment of a powder with a gas; and this does not readily lend itself to a continuous process, owing to the fact that a powder cannot be introduced or withdrawn through a gas-tight trap, as can be done with a liquid. On the other hand, it has been found, in accordance with the present invention, that there are chemical factors which can be so utilized in an appropriate continuous process as to overbalance the disadvantages inherent in continuous treatment of a powder with a gas. These chemical factors will now be pointed out.

The rate of reduction of cupric and cuprous oxides,  $\text{CuO}$  and  $\text{Cu}_2\text{O}$ , increases with temperature, but the resulting copper cake powder becomes increasingly harder as the temperature of reduction rises. Of course, a hard cake is undesirable because of the difficulty of breaking it into powder. Furthermore, too high reduction temperature causes a high rate of reduction on top of the layer of oxide, with little or no reduction on the bottom of the layer. For most purposes the best compromise between these conflicting factors is to employ a temperature between 450° and 550° C. This is true both for batch and continuous processes, although it may be pointed out at this time that continuous operation enables the temperature to be controlled more ad-

vantageously, as well as permitting the material treated to be raised more quickly to proper reducing temperature, and subsequently cooled more rapidly and economically below the atmospheric oxidation point.

When a reducing gas is used which contains both carbon monoxide and hydrogen, a number of reactions occur:



The reduction of the oxides of copper is added, catalytically, by the presence of free copper and is retarded, catalytically, by the presence of water vapor in the gas. At temperatures around 200° C., the inhibiting action of water vapor is very pronounced. While such action decreases as the temperature rises, it is a factor to be reckoned with at 400° C., and even at 450° to 550° C.

Accordingly, reactions (1) and (3) catalyze themselves, while reactions (2) and (4) inhibit themselves. Reaction (5) takes place readily at 450° to 550° C., particularly in the presence of a catalyst so that while CO is present in the gas in any considerable concentration, the water formed is largely eliminated.

These facts, coupled with the mass action laws, make it especially desirable to carry out the reduction countercurrent. The fresh reducing gas with maximum content of CO and H<sub>2</sub> and a minimum content of H<sub>2</sub>O strikes the nearly reduced oxide when the tendency for the reversible reactions:



to proceed to the right is a maximum according to the mass action law in view of the fact that, at such time the ratios Cu : CuO and Cu : Cu<sub>2</sub>O are very high. The presence of the reduced copper also aids in overcoming the normal tendency of the mass action law to retard further reduction.

Due to reaction (5), mentioned above, the water vapor does not reach seriously high concentrations until after the gas and powder have moved countercurrent a considerable distance and the ratio of Cu : CuO or Cu : Cu<sub>2</sub>O has dropped to the point at which mass action law ceases to be an important factor, so far as the solid components of the reactions are concerned.

The heats of reaction are such that when a reducing gas containing both CO and H<sub>2</sub> are brought into contact with copper oxides at 450° to 550° C., there is a strong tendency for the CO to be converted into CO<sub>2</sub> before appreciable amounts of water vapor are formed. The heats of oxidation of copper, carbon monoxide and hydrogen are as follows:

|          | Calories |
|----------|----------|
| Cu + O   | 34,900   |
| 2 Cu + O | 39,900   |
| CO + O   | 67,960   |
| 2 H + O  | 57,826   |

Consequently, if a gas containing both carbon monoxide and hydrogen is brought into countercurrent contact with copper oxides, the latter will pass first through a zone in which the hydrogen is the chief reducing agent and then through a zone in which carbon monoxide is the chief reducing agent.

Methane and hydrocarbons generally are less

readily oxidized than CO and H<sub>2</sub>, so that, if the reducing gas used has any considerable hydrocarbon content, a part of the gas may to advantage be recirculated to give the residual hydrocarbons time to be oxidized, preferably after cooling it to condense the greater part of its water vapor content.

While it is usually advisable (safer and cheaper) to use as the reducing gas carbon monoxide or a mixture of carbon monoxide and hydrogen (water or producer gas), whether enriched by the addition of hydrocarbons (city gas) or not, the process can be carried out using hydrogen alone. In the last case it will be especially advantageous to use an excess of gas, cool to condense the water vapor formed and then recirculate.

As in the case of the batch process, it is ordinarily advisable to use a mixture of cuprous and cupric oxides, the proportions usually ranging from 60 to 90% Cu<sub>2</sub>O, with a complementary amount of CuO, allowance being made for the free copper present with the oxides. Some free copper will ordinarily be present with the oxides (before reduction is started), and the amount of such free copper may be after the order of 5%. The best proportions of cuprous and cupric oxides are dictated by the character of product desired.

One suitable form of apparatus for carrying out the improved process is illustrated diagrammatically, by way of example, in the accompanying drawings, in which:

Fig. 1 is a longitudinal vertical section through the muffle furnace in which the reduction takes place;

Fig. 2 is a side elevation of the cooling section of the apparatus;

Fig. 3 is a section on the line 3—3 of Fig. 1;

Fig. 4 is a detail view of the feed end of the muffle furnace with water extracting apparatus connected thereto;

Fig. 5 is a detail section on the line 5—5 of Fig. 2;

Fig. 6 is a detail section on the line 6—6 of Fig. 2; and

Fig. 7 is a detail section on the line 7—7 of Fig. 6.

The apparatus comprises two main parts, a heating and reducing section (shown in Fig. 1) and a cooling section (shown in Fig. 2). In the first section the mixed oxides are heated to around 450° to 550° C. in a reducing atmosphere to convert the oxides into metallic copper, and in the second section the metallic copper is cooled in a nonoxidizing atmosphere down to a temperature at which the copper may be exposed to air without substantial oxidation taking place.

Running through both sections of the furnace is a flat steel belt 10 passing over pulleys 11, 11, one of which is driven by any suitable means not shown. Preferably, the bearings of one pulley are movable and are biased to tension the belt. The upper half of the belt is wholly enclosed in a flattened steel casing designated as a whole by 12, open at both ends and composed of a plurality of sections which are bolted and welded together. The tube 12 may be considered as having four operating zones or sections 12a, 12b, 12c, and 12d. The feed end 12a of this casing is provided with a hopper 13 for mixed oxides. A vertically adjustable gate 14 regulates the thickness of the layer of oxides carried forward by the belt and also serves to some extent as a closure to prevent escape of reducing gas or entry of atmospheric

air, according to the manner in which the apparatus is operated. Some gas can and will pass in or out through the interstices of the powder on the belt, according to the relative pressure in and outside the casing.

After leaving the hopper the belt passes under a series of pivotally supported weighted bars 15 (see also Fig. 3 which serve to form furrows in the oxide layer for the dual purpose, first of aiding the reduction, and second of rendering the friable mass of reduced copper more easily broken and pulverized.

Attached to the casing section 12a above the bars 15 is a flue 16 for the discharge of spent reducing gases. The adjoining portion 12b of the casing forms the inner chamber of a muffle furnace. Surrounding this section of the casing is an outer heating chamber, the walls 11 of which are formed of fire-brick and covered with a layer of asbestos 17a. As the furnace roof is arched, the top of the casing section 12b is correspondingly arched, as shown in Fig. 3.

Beneath the furnace section 12b is a series of gas heating jets 18 and cooling air jets 18a, both thermostatically controlled by a series of pyrometers 20, 21, 22 and 23, so as to maintain the temperatures within the casing at these four points at around 425° to 450° C., 450° to 500° C., 475° to 550° C., and 400° to 425° C., respectively. These temperatures are given more as a general guide for average operation and not as fixed ranges never to be departed from. Thus, where slow reduction is desired, the temperatures may be reduced, and vice versa.

Beyond the furnace section is the gas-introducing and gas-preheating section 12c, to which is connected a pipe 24 for supplying thereto city or other suitable reducing gas. In addition to the pipe 24, other pipes, as 25 and 26, may be used to supply further amounts of reducing gas direct to the furnace section 12b.

Ordinary coal gas contains preponderating proportions of hydrogen and methane and only a small amount of carbon monoxide. Such gas is not as suitable as city gas composed in part of water gas and hence having a high proportion of carbon monoxide. A gas of this type which has been found to give good results has the following approximate composition:

|                                   | Per cent |
|-----------------------------------|----------|
| Carbon monoxide                   | 32       |
| Hydrogen                          | 33       |
| Methane                           | 12       |
| Other hydrocarbons                | 8        |
| Nitrogen and carbon dioxide, etc. | 15       |
|                                   | 100      |

The gas-introducing section 12c is connected to the cooling section 12d by a gate valve 29 comprising a vertically slidable gate 30 (Fig. 6) which may be raised and lowered by turning the hand-wheel 31 at the upper end of a threaded rod 32. The gate is set so that it just clears the layer of reduced copper on the belt 10 and thereby acts as a constriction in the casing to prevent flow of gas therewith at that point. The cooling section is provided with one or more water jackets 33, so that by the time the reduced copper on the belt 10 reaches the discharge end of the casing 70 it is below the temperature of active oxidation in contact with air.

At the end of the cooling section 12d adjacent the gate valve is an inlet pipe 34 for some suitable non-oxidizing gas, such as air which has 75

been deoxidized by burning oil in it or by passing it over red hot coke or the like. Such gas is often referred to as "DX" gas. It may be slightly reducing, which is preferred for the present purpose. Alternatively, an actively reducing gas may be used, such as ordinary city gas. Also, a part or all of the spent reducing gas passing up the flue 16 may be supplied to the pipe 34, but it is first preferably cooled below 70° C.

10 The non-oxidizing gas flows along the cooling section in the same direction as the belt moves therethrough and is drawn off through a flue 35 adjacent the discharge end of the casing.

As the belt 10 passes over the pulley 11 it contacts with one edge of a hopper 36 and the reduced copper is thereby scraped off and discharged into a saw tooth crusher, not shown.

Especially when the reducing gas is high in hydrogen, it may be desirable to increase the flow of reducing gas, so that when it nears the discharge flue 16 it has been only partially oxidized, and recirculate a part of the gas after passing it through a condenser to eliminate the greater part of the water vapor therein. An attachment for recirculating a part of the reducing gases after condensing out the majority of the water is shown in Fig. 4. A centrifugal blower 40 draws gas from the casing section 12a through pipe 41 and discharges it through condenser 42 and pipe 43 back to the gas inlet pipe 24. A valve-controlled by-pass 44 enables the amount of gas re-circulated to be regulated.

Good results have been obtained with a muffle furnace section 35 feet long, a cooling section of 18 feet, and a belt speed of 5 to 20 feet per hour, depending on the rate of flow of the reducing gases, depth of oxide layer on the belt, temperature in the reducing zone, and other factors. An average speed under present commercial practice is 8 feet per hour. Changing the rate of reduction has a marked influence on the properties of the finished product. Slow reduction gives lower density, finer particle size and lower flow than rapid reduction.

35 In operating the apparatus reducing gas is introduced through the pipe 24, flows counter-current to the direction of movement of the belt 10 through casing sections 12c and 12b and is discharged up the flue 16. As the spent gas inevitably contains small amounts of carbon monoxide, it is desirable to apply sufficient suction to the tube 16 so that the gaseous pressure at the bottom of the flue is slightly below atmospheric and some air is drawn in under the gate 14. For the same reason, it is desirable to put slight suction on the flue 35 to prevent any non-oxidizing gas passing out into the room where the apparatus is located. To this end flues 16 and 35 may be connected to a chimney which is heated to produce a draft. In addition, or in the alternative, suction may be produced by eductor jets 16a and 35a. Butterfly valves 16b and 35b provide further control.

65 The mixed oxides passing through the casing sections 12b and 12c are first heated to the temperature of reduction, then pass through a zone in which hydrogen is the chief reducing agent, next through a zone in which carbon monoxide is the chief reducing agent and finally through a zone in which the hot reduced copper preheats the reducing gases.

In compliance with the patent statutes, the best known forms of the invention have been disclosed, but it will be understood that the disclosure is illustrative and not limiting.

What I claim is:

1. An apparatus for producing a friable mass of copper, comprising an endless moving belt, a tubular casing surrounding the upper section of the belt, means for depositing a layer of copper oxides on the belt at the feed end of the casing, gas discharge flues adjacent each end of the casing, a constriction near the middle of the casing for preventing the flow of gas along the casing at that point, means for introducing reducing gas on the feed side of such constriction for countercurrent flow with respect to the movement of oxides by the belt, means for introducing non-oxidizing gas on the discharge side of such restriction for flow in the same direction as the movement of the belt, and means for cooling the reduced copper on the belt between such constriction and the discharge end of the casing.

2. In the art of reducing copper oxides by causing a continuous ribbon-like stream of the comminuted oxides to travel horizontally and uninterruptedly through a furnace and thence, without change of form or direction, through a cooling chamber that is in communication with the furnace, the improvement which consists in supplying reducing gas to the furnace and causing it to make contact with the oxides in the furnace and to move horizontally counter-current to the direction of travel of the oxide stream; in applying to the furnace, at selected intermediate points along its length, means for establishing within the furnace in connection with the reaction heat inside the furnace, different selected temperatures at such selected intermediate points, and controlling the temperature-establishing means by means responsive to fluctuations in the temperatures, to compensate for such fluctuations, whereby those temperatures are substantially maintained despite variations in reaction heat; in supplying non-oxidizing gas to the cooling chamber and causing it to travel in the same direction as the oxide stream; and in substantially preventing the movement of gas from the furnace into the cooling chamber and from the cooling chamber into the furnace.

3. The method of producing a friable mass of metallic copper, comprising passing a continuous horizontally moving stream of reducing gas over a continuous longitudinally scored ribbon-like stream of heated copper oxides moving horizontally in the opposite direction, and thereafter causing the stream of copper to travel within a stream of cool non-oxidizing gas moving in the direction of travel of the copper stream, while preserving the cross-sectional dimensions of the stream throughout its travels.

4. An apparatus for producing a friable mass of copper, comprising an endless moving belt whose upper course is disposed and travels horizontally, a tubular casing surrounding the upper course of the belt, means for supplying to the upper course of the belt, before it enters the casing, a layer of copper oxides; a gas outlet flue at said end of the casing, means located between the flue and the oxide supplying means for regulating the thickness of the layer so deposited on the belt, means for automatically maintaining different selected temperatures in different portions of the length of the casing adjacent its feed end, means for cooling a section of the casing adjacent its discharge end, means for maintaining a reducing atmosphere in the first named section of the casing, means for maintaining a cooling and non-oxidizing atmos-

phere in the second section of the casing, and means to prevent mingling of the two atmospheres.

5. An apparatus for producing a friable mass of copper, comprising an endless moving belt whose upper course is disposed and travels horizontally, a tubular casing surrounding the upper course of the belt and comprising a furnace section into which the upper course of the belt first enters, and a communicating cooling section into which the belt passes as it leaves said furnace section, means for depositing a layer of copper oxides on the belt at the outer end of the furnace section, means for removing reduced copper from the belt at the outer end of the cooling section, a gas discharge flue at the outer end of the furnace section, a gate located between said flue and the layer-depositing means, movable towards and from the belt to regulate the depth of the layer entering the furnace section, a second gate located at the junction between the furnace and cooling sections and adjustably fixed to permit clearance of the oxide stream while offering an impediment to the movement of gas between the furnace and cooling sections, and means for introducing reducing gas into the inner end of the furnace section and on the furnace side of said second named gate.

6. An apparatus for producing a friable mass of copper, comprising an endless moving belt whose upper course is disposed and travels horizontally, a tubular casing surrounding the upper course of the belt and comprising a furnace section into which the upper course of the belt first enters, and a communicating cooling section into which the belt passes as it leaves said furnace section, means for depositing a layer of copper oxides on the belt at the outer end of the furnace section, means for removing reduced copper from the belt at the outer end of the cooling section, a gas discharge flue at the outer end of the furnace section, a gate located between said flue and the layer-depositing means, movable towards and from the belt to regulate the depth of the layer entering the furnace section, a second gate located at the junction between the furnace and cooling sections and adjustably fixed to permit clearance of the oxide stream while offering an impediment to the movement of gas between the furnace and cooling sections, means for introducing reducing gas into the inner end of the furnace section and on the furnace side of said second named gate, means for introducing cooling gas into the inner end of the cooling section and on the cooling section side of said second named gate, and a gas discharge flue at the outer end of the cooling section.

7. An apparatus for producing a friable mass of copper, comprising an endless moving belt whose upper course is disposed and travels horizontally, a tubular casing surrounding the upper course of the belt and comprising a furnace section into which the upper course of the belt first enters, and a communicating cooling section into which the belt passes as it leaves said furnace section, means for depositing a layer of copper oxides on the belt at the outer end of the furnace section, means for longitudinally scoring the layer so deposited, means for removing reduced copper from the belt at the outer end of the cooling section, a gas discharge flue at the outer end of the furnace section, a gate located between said flue and the layer-depositing means, movable towards and from the belt to regulate the depth of the layer entering the furnace section, a second gate

located at the junction between the furnace and cooling sections and adjustably fixed to permit clearance of the oxide stream while offering an impediment to the movement of gas between the furnace and cooling sections, and means for introducing reducing gas into the inner end of the furnace section and on the furnace side of said second named gate.

8. A reducing furnace of the kind described, comprising a horizontally disposed tubular casing section with an endless belt having its upper course moving horizontally through the casing section, means for depositing a layer of copper oxides on the upper course of the belt before it enters the casing section, a gate at the feed end of the casing section permitting the layer so deposited to pass it, but obstructing the movement of gas outwardly from the casing section, means for introducing reducing gas at the other end of the casing section, a flue at the said feed end of the casing section for causing movement of the gas counter-current to the travel of the belt, means for heating the casing section located at different intermediate points along its length, and means for cooling the casing section located at different intermediate points along its length, said heating and cooling means being thermostatically controlled substantially as and for the purposes set forth.

9. The method which comprises passing a continuous ribbon-like stream of comminuted copper oxides horizontally and slowly through a horizontally disposed furnace in an atmosphere of reducing gas, applying to the furnace at selected intermediate points along the length of the furnace, means for establishing within the furnace in connection with the reaction heat inside the furnace, different selected temperatures at such selected intermediate points, and controlling the temperature-establishing means by means responsive to fluctuations in the temperatures, to compensate for such fluctuations, whereby those temperatures are substantially maintained despite variations in reaction heat.

10. The method which comprises passing a continuous ribbon-like stream of comminuted copper oxides horizontally and slowly through a horizontally disposed furnace in an atmosphere of reducing gas moving countercurrently to the oxide stream, applying to the furnace at selected intermediate points along the length of the furnace, means for establishing within the furnace in connection with the reaction heat inside the furnace, different selected temperatures at such selected intermediate points, and controlling the temperature-establishing means by means responsive to fluctuations in the temperatures, to compensate for such fluctuations, whereby those temperatures are substantially maintained despite variations in reaction heat.

11. The method which comprises passing a continuous ribbon-like stream of comminuted copper oxides horizontally and slowly through a horizontally disposed furnace in an atmosphere of reducing gas moving countercurrently to the oxide stream, applying to the furnace at selected intermediate points along the length of the furnace, means for establishing within the furnace in connection with the reaction heat inside the furnace, different selected temperatures at such selected intermediate points, controlling the temperature-establishing means by means responsive to fluctuations in the temperatures, to compensate for such fluctuations, whereby those temperatures are substantially maintained despite variations in

reaction heat, and thereafter causing the stream of copper to travel, without change of form or direction, within a stream of cool non-oxidizing gas moving in the direction of travel of the copper stream.

12. Apparatus of the kind described comprising, a tubular horizontally disposed casing with an endless belt having its upper course moving horizontally in the casing, means for continuously supplying copper oxides to said belt the casing being divided into a furnace section and a cooling section in communication with each other, the upper course of the belt entering the furnace section and emerging from the cooling section, means for introducing reducing gas at the junction of the two sections and positively causing it to move towards and discharge from the outer end of the furnace section, means for establishing within the furnace section, at selected intermediate points along its length, different selected temperatures at such selected intermediate points, means responsive to fluctuations in the temperatures to compensate for such fluctuations and maintain the temperatures substantially constant, and means for introducing non-oxidizing gas at the junction of the two sections and positively causing it to move towards and discharge from the outer end of the cooling section.

13. The method which comprises passing a continuous ribbon-like stream of comminuted copper oxides horizontally and slowly through a horizontally disposed furnace in an atmosphere or reducing gas moving countercurrently to the oxide stream, applying to the furnace, at selected intermediate points along the length of the furnace, means for establishing within the furnace in connection with the reaction heat inside the furnace, different selected temperatures within a range of about 425° C.-550° C. at such selected intermediate points, and controlling the temperature-establishing means by means responsive to fluctuations in the temperatures, to compensate for such fluctuations, whereby those temperatures are substantially maintained despite variations in reaction heat; the depth of the copper stream, the speed of its travel, and the rate of flow of the gas being chosen each in view of the others, whereby effective reduction of a maximum amount of material may be accomplished in a given time.

14. The method which comprises passing a continuous ribbon-like stream of comminuted copper oxides horizontally and slowly through a horizontally disposed furnace in an atmosphere of reducing gas moving countercurrently to the oxide stream, applying to the furnace, at selected intermediate points along the length of the furnace, means for establishing within the furnace in connection with the reaction heat inside the furnace, different selected temperatures within a range of about 425° C.-550° C. at such selected intermediate points, controlling the temperature-establishing means by means responsive to fluctuations in the temperatures, to compensate for such fluctuations, whereby those temperatures are substantially maintained despite variations in reaction heat; the depth of the copper stream, the speed of its travel, and the rate of flow of the gas being chosen each in view of the others, whereby effective reduction of a maximum amount of material may be accomplished in a given time; and thereafter continuing to move the metal stream and subjecting it to the action of a stream of non-oxidizing gas moving in the direction of travel of the metal stream.

15. A reducing furnace of the kind described comprising a horizontally disposed tubular casing with an endless belt having its upper course moving horizontally through the casing, means for depositing a layer of copper oxides on the upper course of the belt before it enters the casing, means for introducing reducing gas at the other end of the casing and discharging such gas at the feed end of the casing, means for establishing temperature conditions inside the furnace, and means responsive to temperature fluctuations inside the furnace, controlling said temperature-establishing means to compensate for such fluctuations, whereby temperature conditions established inside the furnace may be substantially maintained despite variations in reaction heat. 15.

16. The method which comprises passing a continuous ribbon-like stream of comminuted

5 copper oxides horizontally and slowly through a horizontally disposed furnace in an atmosphere of reducing gas, applying to the furnace at selected intermediate points along the length of the furnace, heating and cooling means for establishing within the furnace in connection with the reaction heat inside the furnace, different selected temperatures at such selected intermediate points, and controlling the temperature-establishing means by means responsive to fluctuations in the temperature, to compensate for such fluctuations, whereby those temperatures are substantially maintained despite variations in reaction heat.

HARRIET L. HALL,  
*Executrix of the Estate of Everett J. Hall,  
Deceased.*